

# UNITED STATES PATENT OFFICE.

GEORG RUDOLPH, OF ELBERFELD, GERMANY, ASSIGNOR TO FARBFENFABRIKEN VORM.  
FRIEDR. BAYER & CO., OF ELBERFELD, GERMANY, A CORPORATION OF GERMANY.

## PRODUCTION OF EFFECTS ON MIXED GOODS COMPOSED OF COTTON AND WOOL.

No. 873,613.

Specification of Letters Patent.

Patented Dec. 10, 1907.

Application filed April 18, 1907. Serial No. 368,987.

*To all whom it may concern:*

Be it known that I, GEORG RUDOLPH, citizen of the German Empire, residing at Elberfeld, Kingdom of Prussia, Germany, have invented new and useful Improvements in Production of Effects on Mixed Goods Composed of Cotton and Wool, of which the following is a specification.

It has hitherto not been possible to dye half-woolen goods with sulfur coloring matters in such a way that the wool fiber remained undyed. I have now discovered that wool after treatment with chromium compounds loses almost completely its affinity for sulfur dyes. On dyeing with sulfur dyes mixed fabrics consisting of cotton and wool in which the wool has been treated with chromium compounds, the wool will remain practically white and it may be dyed afterwards with suitable coloring matters. The wool may be dyed and mordanted before spinning or weaving with cotton. Cotton cloth with white or colored woolen threads *e. g.* a cotton cloth with white or colored edges or lists can thus be obtained.

For the dyeing with sulfur colors it is advisable, to employ a method which does not impair the strength of the animal fiber. For this purpose the process of dyeing may be used which is described in German Letters Patent 173685 and according to which the mixed goods are dyed in a dye bath containing the sulfur dye, sodium sulfid and salts of organic acids possessing a reducing action *e. g.* formic acid, lactic acid, or the like. Such a dye bath is not detrimental to the wool and the protecting action of the chromium compounds is further increased by the lactic acid etc.

White effects can be obtained *e. g.* by using chrome-mordanted wool as list-yarn for cotton piece-goods and dyeing the mixed goods as above stated. Mixed colored effects can be obtained by dyeing wool, chroming it after dyeing, weaving or spinning the dyed and chrome-mordanted wool with cotton yarn and finally dyeing the goods with sulfur colors; or the white chrome-mordanted wool is interwoven, the tissue dyed with sulfur-dyes and the chromed wool is then dyed with suitable dyestuffs.

In carrying out the process practically I can proceed as follows: 10 kilograms of wool are treated for  $1\frac{1}{2}$  hours with 50 grams of potassium bichromate and 100 grams of sulfuric acid or with 50 grams of potassium bichromate, 50 grams of lactic acid and 50 grams of sulfuric acid. It is rinsed, dried and then either spun or interwoven with cotton. The fabric is then dyed in a dye bath charged per 200 liters with

|           |                                        |
|-----------|----------------------------------------|
| 830-1200  | grams of Katigen black TW extra,       |
| 1600-2400 | " " crystallized sodium sulfid,        |
| 1600      | " " caustic soda,                      |
| 3000      | " common salt,                         |
| 5200-6800 | " the acid sodium salt of lactic acid. |

The goods are entered at 20—25° C and dyed for from 1 to  $1\frac{1}{2}$  hours at this temperature, rinsed in water and then in a dilute acetic acid solution. Instead of chroming the wool fabric by itself, it can be chromed after having been spun or interwoven with cotton. In both cases black cotton cloth with white effects is obtained. Of course other sulfur coloring matters can be used. To obtain mixed colored effects the wool before or after chroming may be dyed with suitable coloring matters, *e. g.* anthracene yellow C, acid anthracene red 3 B, benzo fast red FC, brilliant wool blue B extra, al-kali fast green 3 G extra. This may be done either before the spinning or weaving with cotton or after, and in the latter case before or after the dyeing with the sulfur coloring-matters. Variegated effects can be obtained on using wool dyed in different colors.

I do not confine myself to the particulars given in the above example which are merely typical and can be varied within wide limits without altering thereby the nature of the above invention.

Having now described my invention and in what manner the same is to be performed, I declare that what I claim is:—

1. The process of producing variegated colored effects on fabrics composed of cotton and wool, which consists in chroming the wool and then dyeing the fabric with sulfur dyes, the chromed wool resisting the action thereof and remaining uncolored, substantially as described.

2. The process of producing variegated colored effects on fabrics composed of cotton

2  
and wool, which consists in chroming the wool, and then dyeing the fabric with sulfur dyes, the chromed wool resisting the action thereof and remaining uncolored; and then dyeing the fabric with any of the colors ordinarily employed for wool dyeing, substantially as described.

In testimony whereof I have hereunto set my hand in the presence of two subscribing witnesses.

GEORG RUDOLPH. [L. S.]

Witnesses:

OTTO KÖNIG,

J. A. RITTERSHAUS.